

BEST AVAILABLE COPY  
United States Patent Office

3,679,541

Patented July 25, 1972

1

3,679,541

SHEATH/CORE BICOMPONENT FILAMENTS AND  
PROCESS OF PREPARING SAME

Anthony Charles Davis, Pontypool, and Ian Stuart Fisher,  
Harrogate, England, assignors to Imperial Chemical  
Industries Limited, London, England

No Drawing. Filed July 20, 1970, Ser. No. 56,667  
Claims priority, application Great Britain, July 28, 1969,  
37,789/69

Int. Cl. D01d 5/28

U.S. Cl. 161—175

8 Claims

ABSTRACT OF THE DISCLOSURE

Sheath/core bicomponent filaments having a core derived from a fibre-forming linear polyamide or copolyamide and a sheath derived from a copolyester or copolyamide containing poly (alkylene oxide) radicals.

This invention relates to bicomponent filaments having soil-release, anti-soil redeposition and antistatic properties, these properties being durable throughout conventional textile processing and subsequent use.

Processes for improving the hydrophilic properties of polyamide textile materials are well known. For example, surface treatments by hydrophilic coatings have been proposed; however, none of these have been entirely satisfactory since they have either lacked durability or have adversely affected fabric handle.

Homofilaments comprising copolymers containing hydrophilic components have also been suggested. In most cases, the introduction of the hydrophilic component has adversely affected the tensile properties or decreased the resistance to degradation by heat and light.

In yet another prior art method, filaments have been produced from polyamide polymers having hydrophilic additives dispersed therein. The hydrophilic properties of such filaments, although good initially, deteriorate with treatments such as repeated washing due to leaching out of the additive.

We now provide a process by means of which filaments may be produced having adequate tensile properties and resistance to degradation for all normal fibre uses and at the same time having good antistatic and soil-release properties which remain throughout conventional textile processing treatments and subsequent use including repeated washing and cleaning treatments.

According to the present invention we provide a process for the preparation of a bicomponent filament by the extrusion of two streams of different molten polymers in sheath/core relationship, the core being derived from a fibre-forming linear polyamide or copolyamide and the sheath being derived essentially from a copolyester or copolyamide containing poly (alkylene oxide) radicals in an amount such as would result from the reaction of not less than 5 parts by weight of poly (alkylene oxide) per 100 parts by weight of the final copolyester or copolyamide, allowing the conjugate stream to solidify to form a filament and subsequently drawing. Our invention also includes sheath/core bicomponent filaments made according to the process of our invention.

The core may be derived from any fibre-forming linear polyamide or copolyamide, including, for example, poly (hexamethylene adipamide) or poly (caproamide).

The sheath is derived essentially from a copolyester or copolyamide containing poly (alkylene oxide) radicals. Of course, other polymeric constituents may additionally be present in the sheath.

Suitable copolymers are those based on a simple glycol, a dicarboxylic acid and a poly (alkylene oxide).

2

Examples of simple glycols are those of the form  $\text{HO}(\text{CH}_2)_n\text{OH}$ , wherein  $n$  is not less than 2 and not greater than 10, and 1:4-bis(hydroxymethyl) cyclohexane. In the term simple glycol we also include more than one simple glycol.

Examples of suitable dicarboxylic acids on which the copolymers of the sheath may be based are terephthalic, naphthalene-2:6-dicarboxylic and 1:2-diphenoxymethane-4:4'-dicarboxylic acids. We also include the use of more than one dicarboxylic acid. Suitable second dicarboxylic acids are, for example, adipic, isophthalic and sulpho-isophthalic acids. The poly (alkylene oxide) should preferably be poly (ethylene oxide) or poly (propylene oxide), having an average molecular weight not less than 1,000 and not greater than 20,000. Preferably the average molecular weight should be not greater than 6,000. The average molecular weight in question is that for distribution of molecular weight of poly (alkylene oxide) as manufactured. It is convenient and preferred to use a poly (alkylene oxide) glycol in the preparation of the copolyester.

When the sheath is a copolyester, it is most practicable to use a copolyester of ethylene terephthalate and poly (oxyethylene) terephthalate.

Copolyamides suitable for the sheath component are based on aliphatic  $\alpha,\omega$ -dicarboxylic acid and a poly (alkylene oxide) diamine with an aliphatic  $\alpha,\omega$ -diamine or an aliphatic  $\omega$ -amino-carboxylic acid or with both.

Examples of aliphatic dicarboxylic acids on which the sheath may be based are adipic acid, pimelic acid and sebacic acid.

Examples of suitable aliphatic diamines are those of the form  $\text{H}_2\text{N}(\text{CH}_2)_n\text{NH}_2$  wherein  $n$  is not less than 4 and not greater than 10.

The amino-carboxylic acid may be in the form of its lactam such as, for example, epsilon-caprolactam.

The proportion of structural units of the sheath component which are derived from poly (alkylene oxide) should not exceed that which would result from the reaction of 60 parts, preferably 40 parts, by weight of poly (alkylene oxide) in the formation of 100 parts by weight of the final copolyester or copolyamide.

In order to avoid spun yarn stickiness, which leads to difficulty in unwinding packages of spun yarn during drawing, it is preferable that the proportion of structural units of the sheath component which are derived from poly (alkylene oxide) is not excessive. This proportion may be greater in the case of a higher molecular weight poly (alkylene oxide) than in the case of a lower molecular weight poly (alkylene oxide).

We have found particularly advantageous the use of sheath component of a copolyester or copolyamide which is fibre-forming and which has an effective melting point not less than 200° C. These conditions favor successful extrusion to form filaments and successful orientation by cold drawing.

The proportion of the conjugate filament cross-section which is composed of the sheath component should be sufficient such that the sheath comprises a major proportion of the filament surface. It may provide an entire sheath about the core, on the other hand such proportions should not be so great that the dye-fastness and light resistance properties are adversely affected. After subjecting the sheath/core filaments of our invention to a dyeing procedure, the resultant filaments may be reduction cleared, according to known techniques. This treatment results in removal of the dyestuff from the sheath of the filaments so that the lack of dye-fastness and the lack of light resistance normally associated with the presence of dyestuff in the material of which the sheath is composed is no longer a problem. On the other hand, the presence of dyestuff

in the core of the filaments ensures the desirable coloured appearance of the filaments and the dyestuff in the core is fast and light resistant. Thus the proportion of the cross-sectional area being composed of the sheath component should be not less than 5% and not greater than 40%, preferably not greater than 33%. Provided these requirements are met, the filaments may be of concentric or eccentric conformation and of circular or non-circular cross-section.

Any convenient method may be used for the formation of the sheath/core filaments of the present invention.

The filaments manufactured according to the process of our invention may be produced by the use of a multi-hole spinneret to form a yarn which may be oriented by cold-drawing according to methods known in the art.

The sheath and core may optionally contain additives commonly present, and in the amounts commonly used, to produce desired effects, for example colouring materials, delustrants, dyeing additives and stabilizers. Such effects may be confined to the sheath or to the core.

The filaments of our invention may be used in all textile uses, as continuous filament or staple fibre alone or in admixture with other filaments or fibres particularly where soil redeposition, antisoiling and antistatic properties are important.

EXAMPLE 1

A core/sheath bicomponent yarn was melt-spun at 275° C. from a laboratory twin barrel hydraulic extruder. The core polymer was 6.6 nylon containing 0.3% TiO<sub>2</sub> and having a relative viscosity of 37 and the sheath polymer was a copolyester formed from a mixture of equal weights of poly (oxyethylene) glycols of 4000 and 6000 mol. wt. (19% by wt. of copolyester), ethylene glycol, and terephthalic acid, containing 0.5% TiO<sub>2</sub> and having an inherent viscosity of 0.68 and containing as antioxidants 0.09% of 2,4-dimethyl-6-methylcyclohexylphenol, 0.09% of triphenyl phosphite. A 5-filament yarn in which the core occupied 40% of the cross-sectional area was wound up at 400 ft./min. and subsequently drawn to a ratio of 5:1 using a snubber pin at 70° C. and a hot-plate at 175° C. The drawn yarn had a denier of 37.3, tenacity 2.5 g./denier and extensibility 11.6%. A control 5-filament yarn spun at 275° C. from the nylon polymer only and drawn under the same conditions had a denier of 35.0, tenacity 5.3 g./denier and extensibility 20.1%.

Each drawn yarn was four-folded and converted to a weft-knitted fabric sample. The fabrics were washed to remove spinning finish and tested as follows:

(a) Samples of fabric were rinsed in 0.15% aqueous potassium bromide solution and dried, and the electrical resistance of a square of the fabric was measured after conditioning to a relative humidity of 65. Results were as follows: bicomponent fabric—8×10<sup>10</sup> ohms; nylon control fabric—above 10<sup>13</sup> ohms.

(b) Samples of fabric were impregnated with 30% of their weight of dibutyl phthalate and given washing treatments of different intensity. The percentage of the original oil applied remaining on the fabric sample were as follows:

| Sample                    | Percent oil retained after—                                           |                                                                       |                                                             |
|---------------------------|-----------------------------------------------------------------------|-----------------------------------------------------------------------|-------------------------------------------------------------|
|                           | 6 min. in<br>0.07%<br>aqueous<br>commercial<br>detergent<br>at 60° C. | 1 hr. in 0.07%<br>aqueous<br>commercial<br>soap solution<br>at 60° C. | 2 hrs. in<br>0.07%<br>aqueous<br>soap solution<br>at 60° C. |
| Bicomponent-fabric.....   | 12.6                                                                  | 10.9                                                                  | 10.2                                                        |
| Nylon control fabric..... | 52.5                                                                  | 29.2                                                                  | 23.2                                                        |

EXAMPLE 2

A 625 denier yarn consisting of 40 core/sheath bicomponent filaments was spun and wound up at 1718 ft./min. using the apparatus described in British patent specification No. 1,100,430. The volume ratio of core to sheath was 80/20. The core component was 6.6 nylon

containing 0.3% TiO<sub>2</sub> and having a relative viscosity of 42, and the sheath polymer was the copolyester used in Example 1. The yarn was cold-drawn to a ratio of 3.21 giving an oriented yarn of denier 209 with a tenacity of 3.3 g./denier and extensibility 41%. A control yarn was spun from a standard nylon melt-spinning unit at 1718 ft./min., using the same nylon polymer, and drawn to a ratio of 3.21 to an oriented yarn of denier 208, tenacity 3.75 g./denier and extensibility 47%. Each yarn was converted to woven fabric and the fabrics were scoured in a detergent/sodium carbonate solution at 60° C. One portion of each fabric was rinsed in distilled water and another in 0.15% potassium bromide solution. Both fabrics were dried and conditioned in air of known relative humidity, and the fabric electrical resistance was measured; with the fabric sample resting on an insulating sheet, the D.C. resistance was measured between concentric circular metal electrodes, resting on the upper surface of the fabric and of such dimensions that the annular gap had an inner diameter of 50.8 mm. and an outer diameter of 58.8 mm. Results were as follows:

|                    | Bicomponent yarn     |                      | Control nylon yarn    |                      |
|--------------------|----------------------|----------------------|-----------------------|----------------------|
|                    | Water<br>rinse       | KBr<br>rinse         | Water<br>rinse        | KBr<br>rinse         |
| Resistance (ohms): |                      |                      |                       |                      |
| 65 R.H.....        | 6×10 <sup>10</sup>   | 5×10 <sup>9</sup>    | 4.6×10 <sup>11</sup>  | 1.2×10 <sup>11</sup> |
| 38 R.H.....        | 7.5×10 <sup>11</sup> | 1.1×10 <sup>11</sup> | >2.0×10 <sup>12</sup> | 2.0×10 <sup>12</sup> |

These results showed the bicomponent yarn to give a substantially more conductive fabric, particularly in the presence of a small amount of ionic impurity.

EXAMPLE 3

A 685 denier yarn consisting of 40 core/sheath bicomponent filaments was spun and wound up at 1068 ft./min. using the apparatus described in British patent specification No. 1,100,430. The volume ratio of core to sheath was 80/20. The polymers used were as in Example 2 except that the weight percentage of mixed polyether glycols was increased to 25% of the total weight of the copolyester. The yarn was drawn over a snubber pin at 90° C. to a ratio of 3.49 to give an oriented yarn of denier 201, having a tenacity of 3.7 g./denier and an extensibility of 56%. A control yarn was also spun and drawn from the nylon polymer only, with the same process conditions, giving a drawn yarn of 210 denier having a tenacity of 4.4 g./denier and an extensibility of 60%.

The two yarns were separately converted to woven fabrics, which were prepared for electrical resistance measurement by scouring and rinsing as in Example 2. The tendency of the scoured fabrics to cling due to electrostatic charge was assessed comparatively by frictional electrification against poly (ethylene terephthalate) fabric; the electrified samples were allowed to cling to an earthed metal plate at 70° to the horizontal and the time for which clinging continued was measured. Measurements were made at two different values of atmospheric humidity, with the following results:

|                              | Bicomponent yarn     |                      | Control nylon yarn   |                      |
|------------------------------|----------------------|----------------------|----------------------|----------------------|
|                              | Water<br>rinse       | KBr<br>rinse         | Water<br>rinse       | KBr<br>rinse         |
| Resistance (ohms):           |                      |                      |                      |                      |
| 65% R.H.....                 | 5.7×10 <sup>9</sup>  | 2.4×10 <sup>9</sup>  | 3.9×10 <sup>11</sup> | 2.1×10 <sup>11</sup> |
| 38% R.H.....                 | 4.1×10 <sup>10</sup> | 1.1×10 <sup>10</sup> | 2.3×10 <sup>12</sup> | 1.7×10 <sup>12</sup> |
| Duration of clinging (sec.): |                      |                      |                      |                      |
| 65% R.H.....                 | 0                    | 0                    | 137                  | 50                   |
| 38% R.H.....                 | 0                    | 0                    | 370                  | 323                  |

The test results showed the bicomponent yarn of this example to possess an electrical resistance two to three

BEST AVAILABLE COPY

3,679,541

5

orders (depending on the ionic content of the yarn samples) below that of control nylon yarn, and to have no tendency towards electrostatic clinging even at the low R.H. of 38%.

EXAMPLE 4

A 3650 denier yarn consisting of 69 core/sheath bicomponent filaments was spun and wound up at 904 ft./min. using the apparatus described in British patent specification No. 1,100,430. The volume ratio of core to sheath was 80/20. The core component was 6.6 nylon containing 0.2%  $TiO_2$  and having a relative viscosity of 45, and the sheath component was the copolyester used in Example 1. The spun yarn was two-folded and drawn and crimped in one operation, giving a bulky yarn containing 138 filaments having a denier of 2334, tenacity 2.34 g./denier and extensibility 41%. The yarn was used to construct a loop pile carpet by tufting into a hessian backing. An adjoining section of carpet was tufted with a standard crimped carpet yarn of the same nylon polymer of 2450 denier. Separate lengths of carpet each incorporating both types of yarn were finished (a) by a detergent/sodium carbonate scour and water rinse, and (b) by dyeing with Duranol blue BN 300 (1% on weight of carpet).

The carpet pieces after drying were given a secondary bessian backing with a latex adhesive and their electrical properties were assessed under defined humidity conditions by resistance testing and static charge generation measurement. Electrical resistance was measured as in Example 2. Static charging propensity was assessed by measuring the body voltage acquired by a person walking on the carpets with shoe soles of either leather or a composition material, and the time for the voltage to decay to half its value was recorded. Results were as follows:

| Yarn type     | Carpet resistance (ohms) |                     | Static charge in walking at 40% R.H. |              |                   |              |                  |              |
|---------------|--------------------------|---------------------|--------------------------------------|--------------|-------------------|--------------|------------------|--------------|
|               |                          |                     | Maximum voltage (kv.)                |              | Decay time (sec.) |              |                  |              |
|               | R.H. 65%                 | R.H. 40%            | Composition sole                     | Leather sole | Composition sole  | Leather sole | Composition sole | Leather sole |
| Bi-component  | $6.1 \times 10^{11}$     | $>2 \times 10^{12}$ | 3                                    | 1.5          | 20                | 20           |                  |              |
| Control nylon | $1.1 \times 10^{12}$     | $>2 \times 10^{12}$ | 4                                    | 2.5          | 25                | 30           |                  |              |

The results showed that the electrical resistance of the bicomponent filament carpet was less than that of a normal nylon carpet, and that static charges generated were smaller and decayed more rapidly, thus lessening the risk of an unpleasant electric shock.

EXAMPLE 5

A 5-filament core/sheath bicomponent yarn was melt-

6

for the copolyamide. Each yarn was cold-drawn to a ratio of 4.0, giving oriented yarns with the following physical properties:

|                   | Denier | Tenacity (g./denier) | Extensibility (percent) |
|-------------------|--------|----------------------|-------------------------|
| Bicomponent yarns | 26.8   | 3.5                  | 43.8                    |
| Copolyamide yarn  | 35.9   | 3.2                  | 39.2                    |
| Nylon 6.6 yarn    | 35.9   | 5.2                  | 59.6                    |

10 Each yarn was knitted into a hose-leg panel, which was scoured in detergent/sodium carbonate solution to remove spinning finish. Tests to determine the electrical and hydrophilic properties were made as follows:

(a) The electrical resistance of a square of fabric was measured after conditioning in an atmosphere of relative humidity 31 or 60.

(b) Squares of fabric were electrified by friction against talc and allowed to cling against a vertical electrically earthed metal surface in an atmosphere at relative humidity 30. The time until the sample dropped away was measured.

(c) Fabric squares were spotted with mineral oil containing a blue dyestuff and immersed in distilled water at 20-25° C. The tendency of oil to be displaced by water is considered to be a measure of the hydrophilic property of the surface.

The behavior of the oil was noted on a 5-point scale as follows:

30 E (excellent)—oil collects into drops which float off the fabric in under one minute

VG (very good)—oil droplets released slowly during 5 minutes

25 G (good)—oil collects into droplets which cling to the fabric

M (moderate)—oily area contracts but does not all collect into droplets

P (poor)—oily areas unchanged or widening.

50 Fabrics were tested for oil-release properties in the scoured state and after 1 hour or 3 hours of washing in 0.4% "Persil" at 60° C.

Test results are shown in the following table.

|                  | Electrical resistance (ohms) |                      | Duration of clinging (sec.) | Hydrophilic properties |              |               |
|------------------|------------------------------|----------------------|-----------------------------|------------------------|--------------|---------------|
|                  | 60% R.H.                     | 31% R.H.             |                             | Scoured                | Washed 1 hr. | Washed 3 hrs. |
| Bicomponent yarn | $2.5 \times 10^{11}$         | $7.0 \times 10^{12}$ | 81                          | VG                     | G-VG         | G-VG          |
| Copolyamide yarn | $2.9 \times 10^{11}$         | $7.0 \times 10^{12}$ | 115                         | VG-                    | VG           | G-VG          |
| Nylon 6.6. yarn  | $6.5 \times 10^{12}$         | $1.0 \times 10^{13}$ | >300                        | M                      | P            | P             |

What we claim is:

1. A sheath/core bicomponent filament in which the core consists of a fibre-forming linear polyamide or copolyamide and the sheath consists of a copolyester containing poly(alkylene oxide) radicals in an amount such as would result from the reaction of not less than 5 parts by weight of poly(alkylene oxide) per 100 parts by weight of the final copolyester.

65 2. A sheath/core bicomponent filament according to claim 1 in which the sheath component occupies no less than 5% and no greater than 33% of the cross-sectional area of the filament.

70 3. A sheath/core bicomponent filament according to claim 1 in which the poly(alkylene oxide) is poly(ethyl-

spun at 310° C. using the apparatus of Example 1 and wound up at 400 ft./min. The core polymer was 6.6 nylon containing no additives and having a relative viscosity of 45. The sheath polymer was a copolyamide prepared from hexamethylenediamine, adipic acid and a diamine prepared from polyoxyethylene glycol of molecular weight 1540 by reaction with thioryl chloride followed by ammonia, substantially as described in British patent specification No. 948,507. The weight proportion of the polyether diamine in the copolyamide was 15%, and the sheath occupied 40% of the cross-sectional area. Control 5-filament yarns were spun using a single-barrel extruder from the separate polymers alone, with a melt temperature of 292° C. for the 6.6 nylon homopolymer and 290° C.

75 claim 1 in which the poly(alkylene oxide) is poly(ethyl-

ene oxide) having an average molecular weight in the range 1,000 to 20,000 inclusive.

4. A sheath/core bicomponent filament according to claim 1 in which the copolyester of the sheath contains poly (alkylene oxide) radicals in an amount such as would result from the reaction of not more than 40 parts by weight of poly (alkylene oxide) per 100 parts by weight of the said copolyester.

5. A sheath/core bicomponent filament according to claim 1 in which the sheath comprises a copolyester of 10 ethylene terephthalate and poly (oxyethylene) terephthalate.

6. A process for the preparation of a bicomponent filament by the extrusion of two streams of different molten polymers in sheath/core relationship, the core being derived from a fibre-forming linear polyamide or copolyamide and the sheath being derived essentially from a copolyester containing poly (alkylene oxide) radicals in an amount such as would result from the reaction of not less than 5 parts by weight of poly (alkylene oxide) per 100 parts by weight of the final copolyester, allowing the 20 conjugate stream to solidify to form a filament and subsequently drawing.

7. A process according to claim 6 in which the sheath

component occupies no less than 5% and no greater than 33% of the cross-sectional area of the filament.

8. A process according to claim 6 in which the copolyester of the sheath contains poly (alkylene oxide) radicals in an amount such as would result from the reaction of not more than 40 parts by weight of poly (alkylene oxide) per 100 parts by weight of the said copolyester.

#### References Cited

##### UNITED STATES PATENTS

|           |         |                 |             |
|-----------|---------|-----------------|-------------|
| 3,594,266 | 7/1971  | Okazaki et al.  | 161—175 X   |
| 3,616,183 | 10/1971 | Brayford et al. | 161—175     |
| 3,632,666 | 1/1972  | Okazaki et al.  | 161—175 X   |
| 3,522,329 | 7/1970  | Okazaki et al.  | 260—857 PEO |
| 3,551,278 | 12/1970 | Ogata et al.    | 161—175     |
| 3,558,419 | 1/1971  | Okazaki et al.  | 161—175     |

ROBERT F. BURNETT, Primary Examiner

R. O. LINKER, JR., Assistant Examiner

U.S. Cl. X.R.

264—171, Dig. 26